

# United States Patent

[19]

Kohler et al.

[11] 3,802,937

[45] Apr. 9, 1974

[54] **PRODUCTION OF CUBE-ON-EDGE  
ORIENTED SILICON-IRON**

[75] Inventors: **Dale M. Kohler; Martin F.  
Littmann, both of Middletown,  
Ohio**

[73] Assignee: **Armco Steel Corporation,  
Middletown, Ohio**

[22] Filed: **Sept. 30, 1966**

[21] Appl. No.: **583,459**

[52] U.S. Cl. .... **148/111, 148/31.55, 148/110,  
148/112**

[51] Int. Cl. .... **H01f 1/04**

[58] Field of Search .... **148/31.55, 110, 111, 112**

[56] **References Cited**

UNITED STATES PATENTS

2,599,340 6/1952 Littmann ..... 148/111

|           |         |                   |           |
|-----------|---------|-------------------|-----------|
| 2,826,520 | 3/1958  | Rickett .....     | 148/111   |
| 2,867,557 | 1/1959  | Crede .....       | 148/111   |
| 3,105,782 | 10/1963 | Walter .....      | 148/111 X |
| 3,305,354 | 2/1967  | Boni et al. ..... | 148/31.55 |
| 3,333,991 | 8/1967  | Kohler .....      | 148/111   |
| 3,333,992 | 8/1967  | Kohler .....      | 148/111   |
| 3,345,219 | 10/1967 | Detert .....      | 148/111   |

Primary Examiner—L. Dewayne Rutledge

Assistant Examiner—W. R. Satterfield

Attorney, Agent, or Firm—Melville, Strasser, Foster & Hoffman

[57] **ABSTRACT**

An improvement in the production of cube-on-edge silicon-iron comprising the step of heating the silicon-iron having an oxygen content no greater than 0.0045 percent to a temperature of from 2,100°F. to not more than 2,400°F. immediately prior to hot rolling.

**8 Claims, No Drawings**

## PRODUCTION OF CUBE-ON-EDGE ORIENTED SILICON-IRON

This invention relates to a method of producing grain-oriented silicon-iron sheet or strip for magnetic purposes. The grain orientation to which this invention refers is that wherein the body-centered cubes making up the grains or crystals are oriented in the cube-on-edge position, designated (110) [001] in accordance with the Miller Indices. More specifically, this invention relates to an improved and economical method of producing grain-oriented silicon-iron, whereby the temperature range to which the silicon-iron is heated prior to hot rolling is lowered by maintaining the oxygen content of the silicon-iron below a critical lower limit.

As is well known, silicon-irons having the (110) [001] orientation are characterized by a relatively high permeability in the rolling direction and a relatively low permeability in a direction at a right angle thereto. A commercial product of this nature has been used successfully for many years for the manufacture of laminations or cores in transformers, generators and the like, because of its low core loss and high permeability in the rolling direction.

The greater part of the cube-on-edge oriented silicon-iron sheet stock is currently made from the raw materials by a number of steps which include melting, refining, casting and hot rolling ingots or slabs of a suitable composition to hot bands usually less than 0.1 inch thick. Following annealing and pickling steps, the material is cold rolled in one or more stages with intermediate anneals, subjected to a decarburizing step, and finally annealed at a temperature high enough to cause secondary recrystallization. The secondary recrystallization has been of the grain boundary energy type.

As indicated above, current practice begins the hot rolling step either with a slab or directly with an ingot. In the first instance an ingot is cast. The ingot is soaked at a high temperature of about 2,200° F. to 2,300° F. for several hours in order to equalize the ingot temperature to obviate problems caused by differential cooling in the ingot. The ingot is then rolled into a slab, generally about 6 inches thick, and allowed to cool slowly. Prior to the hot rolling step, the slab is reheated to about 2,500° to 2,550° F.

When direct hot rolling from an ingot is practiced, it is usual to cast an ingot and soak it at about 2,450° F. prior to the hot rolling step.

The temperature to which a slab is reheated or an ingot is heated prior to the hot rolling step has been the subject of much study among prior art workers. It was taught by Goss in U.S. Pat. No. 2,084,337, issued June 22, 1937, that the ingot should be heated to about 2,000° F. or above, and the reduced slab should be heated to about 2,000° F. Although silicon-iron may be rolled at a temperature as low as 2,000° F., the final product does not exhibit good magnetic qualities.

Littmann and Heck in U.S. Pat. No. 2,559,340, issued June 3, 1952, taught that superior permeabilities could be obtained in silicon-iron by hot rolling from a high initial temperature. They discovered that the magnetic properties of nominal 3 percent silicon-iron would be much improved if the ingot or reheated slab were taken to a temperature above about 2,300° F. and up to about 2,550° F. (or the highest temperature possible without burning) prior to the hot rolling step. As indicated above, this teaching has been adopted univer-

sally by the industry. Such extremely high temperatures, however, have certain serious disadvantages which the industry has attempted for a number of years to overcome. Such high temperatures are difficult to work with, and one of the principal problems is the disposal of slag which forms on the slabs or ingots when they are heated above about 2,400° F. This slag comprises liquid oxide formed by the oxidation of the surface of the slab. Accumulation of this slag eventually interferes with the operation of the slab or ingot heating furnace and it becomes necessary to take the furnace out of operation in order to remove the slag. Because of the dependence of the hot rolling mill on a steady supply of slabs or ingots, the output of the hot mill is severely curtailed each time a furnace is down for repairs. In fact, the production of the entire steel making facility is affected. In addition to costly shutdowns because of slag accumulation, such high temperatures incur higher heating costs, and require more expensive heating equipment. The high temperatures and corrosive effect of the slag greatly reduce furnace refractory life. Nevertheless, all of these disadvantages have been considered unavoidable and the expense entailed thereby has been considered necessary in order to produce silicon-iron of the highest quality.

It was taught by Rickett in U.S. Pat. No. 2,826,520 issued Mar. 11, 1958, that the slag problem could be eliminated by heating the slabs within the limited temperature range of 2,225° F. to 2,275° F. for a minimum of 8 hours. However, this method has not been adopted commercially and the product produced thereby is not characterized by high magnetic qualities.

While all of the work represented by the aforementioned patents concerned so-called critical ranges within the broad general range of slab heating temperatures, for commercially produced silicon-iron alloys containing the standard elements, none was dependent upon nor related to the oxygen content which normally exceeded 0.005 percent, and often was as high as 0.010 percent.

It may be seen from the foregoing discussion of the prior art that there are different and sometimes conflicting teachings as to the most desirable temperatures for the ingot and slab heating steps in the production of grain oriented silicon-iron. It is therefore a primary object of the present invention to provide a method of producing cube-on-edge oriented silicon-iron whereby the slab or ingot temperature prior to the hot rolling step has been rendered nugatory in relation to the quality of the final product.

It is also a primary object of the present invention to provide a more economical method for the manufacture of cube-on-edge silicon-iron whereby savings are realized both in the processing of the material and in the less severe conditions affecting the apparatus or equipment used in its manufacture.

It is an object of the present invention to provide such a method without sacrificing the high standards with respect to the magnetic properties of the final product presently demanded of the industry.

It is an object of the present invention to provide such a method characterized by improved reliability through the use of a combination of processing steps which insure consistently excellent magnetic properties in the final product.

It is an object of the present invention to define the composition of the silicon-iron within limits which

allow its metallurgical structure to be controlled at each step of the process.

These and other objects of the invention which will be set forth hereinafter or will be apparent to one skilled in the art upon reading these specifications are accomplished in those procedures and products of which certain exemplary embodiments will now be described.

In accordance with the present invention, it has been discovered that it is the oxygen level of the silicon-iron, as well as the levels of manganese and sulfur, which determine the optimum ingot or slab heating temperature.

In the production of cube-on-edge silicon-iron there are two basic requirements. First, the proper grain structure and orientation must be achieved after the decarburization step at the final gauge. Secondly, an inhibitor of normal grain growth must be provided in order to promote secondary growth of the decarburized, primary recrystallized structure during the final high temperature anneal. While a number of inhibitors such as manganese selenide may be used, for purposes of an exemplary showing the process of the present application will be described in terms of manganese sulfide as the inhibitor.

It is known that when the manganese sulfide, in the amount formed by having the manganese and sulfur contents in the ranges given below, is well dispersed as submicroscopic precipitates in the silicon-iron, these precipitates will inhibit primary grain growth following recrystallization after cold rolling. Thus, during the final anneal of the material, the secondary grains which start to grow at about 1,700° F. can engulf the primary grains to produce the desired cube-on-edge orientation.

It has been discovered that when the oxygen content of the silicon-iron is kept within the limits given below, a better performance from the manganese sulfide inhibitor is obtainable, and high slab or ingot temperatures are not required. In fact, slab or ingot temperatures may be used which are below what would normally be thought to be the temperature at which the majority of the manganese sulfide would go into solution. The reason for this is not fully understood. While not intending to be bound by theory, it is believed that the silicon-iron of the present invention, having the low oxygen content given below, may naturally give a finer dispersion of the sulfide phase because of the absence of oxide nucleation sites.

In the practice of the present invention, the composition of the silicon-iron is critical. The amount of oxygen should not exceed 0.0045 percent and preferably should not exceed 0.0030 percent. The manganese content should be from about 0.03 percent to about 0.08 percent, and preferably from about 0.045 percent to about 0.065 percent. The lower limit is determined by the amount of manganese necessary to form a sufficient quantity of manganese sulfide to act as a grain growth inhibitor. The upper limit is determined by the solubility of the manganese sulfide prior to hot rolling, the higher manganese causing the sulfide to be less soluble. Also, higher manganese contents render sulfur additions to the silicon-iron at later stages of the processing less effective. Initial sulfur should be present in an amount from about 0.015 percent to about 0.030 percent and preferably from about 0.020 percent to about 0.025 percent. Selenium may be substituted for

sulfur in approximately the same proportions. The initial carbon content should be from about 0.015 percent to about 0.035 percent, and preferably from about 0.020 percent to about 0.030 percent. The silicon content may be from about 1.8 to 4 percent or higher, the lower limit being the minimum silicon which will avoid a phase change to gamma iron upon heating, while the upper limit is dependent upon the ability of the material to be cold rolled without breakage. The nitrogen content should not exceed about 0.007 percent and preferably should not exceed about 0.004 percent. No more than about 0.008 percent total aluminum should be present. It is preferred to have that portion of the aluminum present in the acid-soluble form constitute less than 0.002 percent.

To obtain the critical oxygen content of the present invention, any low oxygen refining process may be used, including vacuum techniques. One process, which has the advantage of being amenable to the use of existing apparatus such as the open hearth or electric furnace, is disclosed by Boni and Heck, U.S. Pat. No. 3,305,354. The re-ladling process of their invention is capable of removing oxygen to a level of about ten parts per million or 0.001 percent.

The silicon-iron having the melt composition given above may be conventionally cast into ingots or it may be continuously cast into slab-ingots. Hereinafter the use of the terms "slabs" and "ingots" is intended to include silicon-iron which has been continuously cast.

Prior to the step of rolling to hot bands, the silicon-iron will be heated whether it be in ingot form (where direct rolling to strip is used) or slab form (where a re-heating step is practiced). In accordance with the present invention, the slabs or ingots are heated to within a temperature range between the lowest temperature at which the ingots or slabs are workable and the highest temperature at which no appreciable amount of slag will be formed. Conventionally the slabs will be held at temperature for a period of less than one hour, while ingots are generally soaked for several hours.

While slabs or ingots are workable in the laboratory at temperatures as low as 1,800° F., it has been found that the lowest practical temperature under plant processing conditions is about 2,100° F.

The highest temperature at which no appreciable amount of slag will be formed is dependent upon a number of factors. These factors include time at temperature, atmosphere, type of flame and the like. Nevertheless, it has been determined that the above described disadvantages obtained when the slabs or ingots are heated to a high temperature before rolling to strip may be avoided if the slab or ingot temperature does not exceed about 2,400° F.

The heated ingots or reheated slabs are then rapidly hot rolled to the desired hot band thickness. In the practice of the present invention, the temperature at which the hot rolling is completed is not considered to be critical in and of itself. It is preferred that the finishing temperature be above 1,650° F. Similarly, the coiling temperature has not been found to be extremely critical. A temperature of about 1,200° F. is normal.

The steps of the process following hot rolling are conventional. The hot band may be annealed before it is cold rolled in order to improve the structure. If an initial anneal is used, the temperature may vary from about 1,650° F. to about 2,000° F., and preferably is

about 1,800° F., for a time of up to about four minutes at temperature.

Oriented silicon-iron having a final thickness of about 0.012 inch is usually cold rolled in two stages with an intermediate open anneal which may be over a broad range of about 1,550° F. to about 1,850° F. The amount of cold reduction in each step will depend largely upon the final thickness desired. While final thickness does not constitute a limitation on the present invention, the teachings herein are particularly applicable to the production of oriented silicon-iron having a final thickness of about 0.014 inch or less.

The silicon-iron will be decarburized to a value of 0.003 percent or less during one or more of the anneals. This may be done in an atmosphere such as wet hydrogen.

After decarburization, the strip is generally coated with an annealing separator and box annealed for at least 8 hours at a minimum temperature of 2,000° F. Higher temperatures and longer times at temperature are used when it is necessary to remove sulfur or other undesirable impurities. The sulfur content will be reduced to less than 0.002 percent during the final anneal.

Various modifications may be made in the processing steps following the hot rolling without destroying the beneficial effects imparted by the particular composition of the silicon-iron and especially its oxygen content. Therefore, it will be understood that the processing of the material beyond the hot rolling stage has been described as exemplary and does not constitute a limitation upon the invention.

When the oxygen content of the silicon-iron, which may be from a trace to 0.0045 percent is in the upper portion of this range, and particularly when it is above about 0.0030 percent, it may be found desirable to heat the ingots or slabs to a temperature within the upper portion of the above given range, i.e. to a temperature from about 2,300° F. to about 2,400° F.

It is a feature of the present invention that the silicon-iron sheet stock may be treated at final gauge, and immediately prior to or during the primary grain growth portion of the final anneal, with sulfur, selenium or their compounds from an external source. The use of sulfur is preferred for economic reasons. The sulfur may be added in the ways taught by Kohler in U.S. Pat. Nos. 3,333,991 and 3,333,992. As taught in these patents the sulfur addition may be made in several ways. For example, sulfur or sulfur-bearing compounds may be added to the annealing separator in the final anneal. Similarly, the annealing atmosphere of the final anneal may be charged with a gaseous sulfur compound providing the atmosphere is in contact with the surfaces of the silicon-iron. In yet another variant, sulfur or sulfur-bearing compounds may be made available at the surfaces of the sheet material during a decarburizing anneal prior to the final anneal.

The practice of the present invention requires accurate melting and accurate chemical analysis. While the degree of accuracy both in melting and in chemical analysis in plant processing is increasing rapidly, it is often not possible to achieve the degree of accuracy in plant processing that is obtainable in the laboratory. It has been found that in some instances the addition of sulfur from an external source will serve as insurance that the silicon-iron of the present invention, when heated within the above given temperature range prior

to hot rolling, will yield a product having excellent magnetic properties. For example, when the oxygen content of the silicon-iron is within the upper part of the above given range, the addition of sulfur from an external source will insure an excellent product even at a slab or ingot heating temperature of 2,100° F.

As a non-limiting example silicon-iron of the above outlined composition in the form of slabs or ingots may be heated within the range of 2,100° F. to 2,400° F. and rapidly rolled to the desired hot band thickness. If an initial anneal is used the temperature may vary from about 1,650° F. to about 2,000° F. for a time of up to about four minutes at temperature. When a final product about 0.012 inch thick is desired, the silicon-iron will be cold rolled in a first stage to an intermediate gauge of about 0.030 inch. This will be followed by an intermediate anneal at about 1,700° F., and a second stage of cold rolling to final gauge. The material may then be decarburized as described above. Sulfur from an external source may be added in any of the ways and in an amount as taught in the above mentioned Kohler patents, and the material will be subjected to a final box anneal at a minimum temperature of 2,000° F. for at least 8 hours. Again, with respect to the final anneal, higher temperatures and longer times at temperatures will be used if it is necessary to remove sulfur or other undesirable impurities.

The addition of sulfur from an external source in the process of the present invention will also serve to insure a product of excellent magnetic qualities when a single stage cold rolling step is used. The process will be substantially the same as that just described except that the desired final gauge is achieved by a single cold rolling stage.

#### EXAMPLE I

Three slabs (hereinafter designated A, B and C) about 6 inches thick were selected from a heat of silicon-iron which had been melted in an open hearth using the previously mentioned method of Boni and Heck to obtain low oxygen. The analysis of the material in the hot rolled condition was: 3.09 percent silicon, 0.055 percent manganese, 0.022 percent sulfur, 0.020 percent carbon, 0.003 percent phosphorus, 0.006 percent aluminum and 0.0020 percent oxygen.

Slabs A, B and C were heated to 2,550° F., 2,400° F. and 2,100° F. respectively and hot rolled so as to have a temperature of about 1,750° F. immediately after the last reduction. The cooling temperature for all three slabs, which was regulated by the amount of water sprayed on the strip, was about 1,200° F. and the hot band thickness was about 0.080 inch. The hot rolled bands were annealed at 1,800° F.

The hot rolled bands were then cold rolled to 0.030 inch, strip annealed at 1,700° F., cold rolled to 0.012 inch, coated with magnesia containing 2 percent sulfur, and box annealed at 2,200° F. for 24 hours. The magnetic properties of samples of the final material, after applying an insulation taken from the front, middle and back of each coil and the averages thereof are given in Table I. The permeabilities were measured at a magnetizing force of ten oersteds and the core losses in watts per pound at 15 and 17 kilogausses at a frequency of 60 cycles per second.

7  
TABLE I

| Slab Number | Slab Temperature | Permeability | Core Losses  |              |
|-------------|------------------|--------------|--------------|--------------|
|             |                  |              | P15;60 w/lb. | P17;60 w/lb. |
| A           | 2350° F.         | 1831         | .575         | .803         |
| B           | 2400° F.         | 1833         | .566         | .793         |
| C           | 2100° F.         | 1823         | .553         | .785         |

It may be seen from the above table that the magnetic properties of the material which had been hot rolled from widely different temperatures are surprisingly comparable. Whereas the permeability of the 2,100° F. material is substantially the same, the corresponding core losses are slightly better than those for material rolled from the higher temperatures. It may be said that the provision of a silicon-iron of an initial composition within the above described limits, and particularly with a very low oxygen content, has made the slab temperature nugatory in relation to the quality of the product. Of course, it is usually better from a cost consideration to use the lowest temperature consistent with mill practices. For instance, when silicon-iron slabs are being heated with slabs of carbon steel or stainless steel, it would be more practical to heat the silicon-iron slabs

The permeability values show that the low oxygen content of the hot rolled band is strongly associated with high permeability. These values also indicate that, as the oxygen content increases, the permeability decreases more rapidly when the initial annealing temperature is lower. Therefore, when the oxygen content falls on the higher side of the desired range, the harmful effects can be partially offset by the use of higher initial annealing temperatures.

## EXAMPLE III

Two slabs about six inches thick representing two ingots were selected at random from each of two heats having ladle analyses as follows:

| Heat Number | %C   | %Mn  | %S   | %Si  | %N    | %O    | %Al (total) |
|-------------|------|------|------|------|-------|-------|-------------|
| A           | .026 | .066 | .023 | 3.21 | .0052 | .0070 | .0053       |
| B           | .025 | .053 | .023 | 3.13 | .0057 | .0023 | .0061       |

to the temperature range dictated by the other materials.

## EXAMPLE II

One slab six inches thick from each of five heats of silicon-iron containing about 3.1 percent silicon was reheated to a temperature of 2,100° F. and hot rolled into coils 0.076 inch thick. Adjacent samples taken from the centers of the hot rolled coils were initially annealed in the laboratory at 1,675° F. and 1,800° F. for about three minutes in air. All of the samples were then processed to a final thickness of 0.012" in two stages of cold reduction.

The samples were annealed at 1,675° F. in hydrogen for about 1 minute at their intermediate thickness of 0.026 inch. After the second cold rolling, they were decarburized at 1,500° F. for about three minutes in wet hydrogen and given a final box anneal at 2,200° F. in hydrogen for 24 hours.

Table II shows the initial compositions and final permeability values for the materials given the two initial annealing temperatures.

TABLE II

| Slab | %C   | %Mn  | %S   | %O    | %N    | 1675° F.<br>Initial Anneal | 1800° F.<br>Initial Anneal |
|------|------|------|------|-------|-------|----------------------------|----------------------------|
|      |      |      |      |       |       | Permeability<br>H = 10     | Permeability<br>H = 10     |
| A    | .022 | .059 | .022 | .0015 | .0057 | 1771                       | 1791                       |
| B    | .023 | .060 | .024 | .0019 | .0057 | 1731                       | 1797                       |
| C    | .016 | .062 | .018 | .0030 | .0030 | 1676                       | 1761                       |
| D    | .019 | .062 | .019 | .0050 | .0054 | 1641                       | 1747                       |
| E    | .023 | .048 | .016 | .0076 | .0074 | 1596                       | 1706                       |

TABLE III

## HEAT A (.0070% O)

| Thickness in Mils | P15;60 w/lb. | P17;60 w/lb. | Perm. H=10.  |
|-------------------|--------------|--------------|--------------|
| 11.0              | .500         | .725         | 1825         |
| 10.3              | .610         | .980         | 1680         |
| 10.2              | .585         | .935         | 1695         |
| 10.5              | .555         | .900         | 1740         |
| 10.5              | .560         | .900         | 1725         |
| 10.6              | .500         | .740         | 1805         |
| 10.5              | .552         | .863         | 1728 Average |

## EXAMPLE V

One slab six inches thick from each of four different heats was reheated to a temperature of 2,100° F. and 5 hot rolled into coils 0.076 inch thick. Samples were taken from the centers of these coils and processed in the laboratory. The samples were annealed at 1,800° F. for about 3 minutes, cold rolled directly to 0.012 inch without an intervening anneal, decarburized in a strip 10 anneal in wet hydrogen at 1,500° F., coated with magnesia with and without sulfur, and box annealed in hydrogen at 2,200° F. for 30 hours. The permeability values obtained are shown below in Table V together with the analyses of the hot rolled samples.

TABLE V

| Slab | %C   | %Mn  | %S   | %O    | %N    | No Sulfur    | 4% Sulfur    |
|------|------|------|------|-------|-------|--------------|--------------|
|      |      |      |      |       |       | Added to MgO | Added to MgO |
| A    | .022 | .059 | .022 | .0015 | .0057 | 1605         | 1770         |
| B    | .022 | .060 | .023 | .0018 | .0057 | 1625         | 1745         |
| C    | .024 | .048 | .017 | .0065 | .0076 | 1552         | 1665         |
| D    | .021 | .069 | .020 | .0090 | .0050 | 1590         | 1632         |

## HEAT B (.0023% O)

| Thickness in Mils | P15;60 w/lb. | P17;60 w/lb. | Perm. H = 10. |
|-------------------|--------------|--------------|---------------|
| 10.6              | .520         | .760         | 1815          |
| 10.4              | .500         | .740         | 1820          |
| 11.0              | .515         | .760         | 1805          |
| 10.5              | .490         | .730         | 1830          |
| 10.2              | .490         | .730         | 1830          |
| 10.3              | .505         | .765         | 1815          |
| 10.5              | .503         | .748         | 1819 Average  |

## EXAMPLE IV

Two slabs about 6 inches thick representing two ingots were selected at random from each of six heats with varying amounts of oxygen. These slabs were heated to a temperature of 2,385° F. or just below the slagging temperature and hot rolled rapidly to hot bands 0.076 inch thick. Samples representing the center of the coils were processed in the laboratory. The hot rolled pieces were annealed at 1,800° F. for about 3 minutes, pickled and cold rolled to an intermediate thickness of 0.022 inch. After a strip anneal for about one minute at 1,750° F., the samples were cold rolled to 0.0088 inch, decarburized at 1,500° F. in wet hydrogen, coated with magnesia and box annealed at 2,200° F. in dry hydrogen for 30 hours. The analyses of the hot bands and the magnetic properties obtained are shown below:

TABLE IV

| Heat | %C   | %Mn  | %S   | %Si  | %N    | %O    | P17;60 w/lb. | Perm. H=10. |
|------|------|------|------|------|-------|-------|--------------|-------------|
| A    | .023 | .070 | .025 | 3.23 | .0060 | .0012 | .639         | 1837        |
| B    | .018 | .061 | .024 | 3.05 | .0067 | .0013 | .657         | 1825        |
| C    | .022 | .047 | .023 | 3.16 | .0061 | .0044 | .666         | 1821        |
| D    | .020 | .052 | .020 | 3.24 | .0056 | .0064 | .730         | 1760        |
| E    | .022 | .069 | .021 | 3.21 | .0052 | .0070 | .90          | 1695        |
| F    | .024 | .044 | .017 | 3.13 | .0070 | .0077 | >.90         | 1675        |

These data clearly show the very strong effect of oxygen content on the texture and magnetic properties obtainable. The core loss values attained for the samples with oxygen below 0.0020 percent are excellent and lower than those hitherto obtainable.

25 These data show that a sulfur addition to the magnesia is rendered more effective when the oxygen content is maintained within the critical range of the invention. The test results for the materials to which sulfur has been added represent excellent magnetic quality, when it is considered that only a single cold reduction was used.

30 35 It will be seen from the above examples that it is possible to attain excellent magnetic properties in the product without heating the slabs or ingots to a temperature range wherein liquid slag is formed.

Modifications may be made in the invention without departing from the spirit of it.

40 The embodiments of the invention in which an exclusive property or privilege is claimed are defined as follows:

45 50 55 1. In a method for producing cube-on-edge silicon-iron having a silicon content of from about 1.8 percent to about 4 percent and processed by steps including hot rolling to intermediate gauge, cold rolling to final gauge, decarburizing and annealing whereby to effect secondary recrystallization favoring growth of cube-on-edge nuclei by grain boundary energy, the improvement comprising in combination therewith the step of heating said silicon-iron having an oxygen content no greater than 0.0045 percent to a temperature of from 2,100° F. to not more than 2400° F. immediately prior to said hot rolling step.

2. In a method for producing cube-on-edge silicon-

65 iron having a silicon content of from about 1.8 percent to about 4 percent and processed by steps including hot rolling to intermediate gauge, cold rolling to final gauge, decarburizing and annealing whereby to effect secondary recrystallization favoring growth of cube on-

edge nuclei by grain boundary energy, the improvement comprising in combination therewith the step of heating said silicon-iron having an oxygen content no greater than 0.0030 percent to a temperature of from 2,100° F. to not more than 2,400° F. immediately prior to said hot rolling step.

3. In a method for producing cube-on-edge silicon-iron having a silicon content of from about 1.8 percent to about 4 percent and processed by steps including hot rolling to intermediate gauge, cold rolling to final gauge, decarburizing and annealing whereby to effect secondary recrystallization favoring growth of cube-on-edge nuclei by grain boundary energy, the improvement comprising in combination therewith the step of heating said silicon-iron having an oxygen content no greater than 0.0045 percent to a temperature of from 2,300° F. to not more than 2,400° F. immediately prior to said hot rolling step.

4. The process claimed in claim 1 wherein said silicon-iron has an initial composition including from about 0.015 percent to about 0.035 percent carbon, from about 0.03 percent to about 0.08 percent manganese, from about 0.015 percent to about 0.030 percent sulfur, 0.007 percent maximum nitrogen, 0.008 percent maximum total aluminum and the balance substantially iron.

5. The process claimed in claim 2, wherein said silicon-iron has an initial composition including from about 0.020 percent to about 0.030 percent carbon,

from about 0.045 percent to about 0.065 percent manganese, from about .020% to about 0.025% sulfur, 0.004 percent maximum nitrogen, .002% maximum acid-soluble aluminum, and the balance substantially iron.

6. The process claimed in claim 2 including the step of reacting said silicon-iron with sulfur from an external source after said cold rolling and prior to said secondary recrystallization whereby to inhibit primary grain growth.

7. In a method for producing cube-on-edge silicon-iron having a silicon content of from about 1.8 percent to about 4 percent and processed by steps including hot rolling to intermediate gauge, cold rolling to final gauge, decarburizing and annealing whereby to effect secondary recrystallization favoring growth of cube-on-edge nuclei by grain boundary energy, the improvement comprising in combination therewith the steps of heating said silicon-iron having an oxygen content no greater than 0.0045 percent to a temperature of from 2,100° F. to not more than 2,400° F. immediately prior to said hot rolling step, and reacting said silicon-iron with sulfur from an external source after said cold rolling and prior to said secondary recrystallization whereby to inhibit primary grain growth.

8. The process claimed in claim 7 wherein said cold rolling step is a single stage reduction to gauge.

\* \* \* \* \*

30

35

40

45

50

55

60

65